

# UNITED STATES PATENT OFFICE.

CARL GRAF, OF COLOGNE-RODENKIRCHEN, GERMANY, ASSIGNOR, BY MESNE ASSIGNMENTS, TO THE CHEMICAL FOUNDATION, INC., A CORPORATION OF DELAWARE.

## PROCESS OF PRODUCING A SURROGATE FOR TANNIN.

1,376,805.

Specification of Letters Patent.

Patented May 3, 1921.

No Drawing.

Application filed March 11, 1916. Serial No. 83,613.

To all whom it may concern:

Be it known that I, CARL GRAF, a subject of the King of Wurttemberg, residing at Cologne-Rodenkirchen, Germany, have invented certain new and useful Improvements in Processes of Producing a Surrogate for Tannin, of which the following is a specification.

The present invention relates to a process 10 of producing a surrogate for tannin, adapted to be employed both alone for itself and also mixed with the extracts of the vegetable tanning materials hitherto employed for the manufacture of leather ready for use, without thereby altering in the least the ordinary manner of working.

The starting material of the process is tar, be it common coal-tar or brown coal-tar, or different kinds of tar extracted from peat 20 or wood. The important elements for the present process are separated from the tar by a preliminary treatment with water or with alkalis, neutral or basic salts or other equivalents. The preliminary treatment 25 with these materials has, compared to that with water, the advantage, that the chief material is better utilized than by treatment only with water. From the tar a liquid will be separated to which sulfates of aluminium 30 and copper are added. In lieu of the sulfate of aluminium we may also use for example, however, the other equivalents such as potassium alum, chrome alum and ammonium alum. The liquid obtained in this way 35 is employed for tanning leather. As a residue a tough, pitch-like mass remains, from which by a repeated treatment with the above-named materials surrogates for tannin may be prepared.

40 It is possible, to introduce in the preliminary treatment the materials to be added in the aftertreatment, such as the sulfates of aluminium and copper. We thereby obtain a product that may, in case of need, also be 45 made use of for tanning leather. The result obtained is, however, less favorable by far than if the materials in question are added only in the after-treatment. It is, furthermore, possible to attain a tanning action by 50 the employment of only one of the sulfates referred to. But, if only sulfate of copper be used, the tanning action is considerably weaker and the leather is less "filled," than will be the case if sulfate of aluminium or any 55 of the sulfates or alums, applicable in its

place be added. On the contrary, by the addition of sulfates of aluminium and the like the liquid is improved to such a degree, that it presents qualities similar to those of extracts of vegetable substances. If, on the contrary, the sulfate of copper be omitted, the leather acquires a dark-gray color, which is, in most cases, not wished for.

The process may be carried out both in the cold and at an increased temperature, it 65 being, however, hastened if the temperature rises.

As an example, in 100 lbs. of water 20 to 25 lbs. of sulfite of soda or equivalent material will be dissolved. To this solution 70 50 lbs. of tar, *e. g.* beech-wood tar are added, when the whole mixture is agitated for some time. Now 8 to 10 lbs. of sulfate of aluminium or 6 to 7 lbs. of alum are added under continuous stirring; the stirring operation 75 is then stopped and 1 to 2 lbs. of sulfate of copper are added, whereupon the stirrer is continued. The liquid obtained by this treatment may at once be employed 80 for tanning or may be inspissated by evaporation.

What I claim is:

1. That process of producing a surrogate for tannin, which comprises treating about 50 lbs. of tar with a solution comprising 100 85 lbs. of water and 20 to 25 lbs. of sulfite of soda or its equivalent; adding and thoroughly mixing with this mixture 8 to 10 lbs. of sulfate of aluminium or its equivalent; adding to the mixture thus obtained 1 to 2 90 lbs. of sulfate of copper.

2. That process of producing a surrogate for tannin, which comprises treating tar with an aqueous solution of an alkali or its equivalent; and thoroughly mixing with the liquid thus obtained a metallic sulfate or mixture of metallic sulfates. 95

3. That process of producing a surrogate for tannin, which comprises treating tar with an aqueous solution of an alkali or its equivalent; separating the liquid thus obtained; and treating said liquid with sulfate of copper and sulfate of aluminium. 100

In testimony whereof I affix my signature in presence of two witnesses.

CARL GRAF.

Witnesses:

T. F. LOUNTS,  
H. HENDEL.